

Dec. 16, 1958

L. S. BUSCH ET AL

2,864,697

TITANIUM-VANADIUM-ALUMINUM ALLOYS

Filed Jan. 23, 1956

2 Sheets-Sheet 1



FIG.1



FIG.2 BY

INVENTORS.  
LEE S. BUSCH,  
GEORGE W. BAUER &  
PAUL E. MOORHEAD  
Grease & Bishop  
ATTORNEYS

Dec. 16, 1958

L. S. BUSCH ET AL

2,864,697

TITANIUM-VANADIUM-ALUMINUM ALLOYS

Filed Jan. 23, 1956

2 Sheets-Sheet 2



FIG. 3



FIG. 4 BY

INVENTORS:  
LEE S. BUSCH,  
GEORGE W. BAUER &  
PAUL E. MOORHEAD  
*Frease & Bishop*  
ATTORNEYS

1

2,864,697

## TITANIUM-VANADIUM-ALUMINUM ALLOYS

Lee S. Busch, George W. Bauer, and Paul E. Moorhead, Warren, Ohio, assignors to Mallory-Sharon Metals Corporation, a corporation of Delaware

Application January 23, 1956, Serial No. 560,512

6 Claims. (Cl. 75—175.5)

The invention relates to titanium-base alloys and more particularly to ternary alloys of titanium with vanadium and aluminum. 15

The increasing use of titanium and titanium alloys has resulted in commercial requirements for a titanium alloy particularly adapted for being rolled into sheet material 20 in which high ductility may be developed to permit forming and in which high strength may be developed after forming. In other words, a need exists for titanium sheet alloy material which may be treated to be highly ductile with excellent forming properties and which thereafter may be aged to provide high strength in the article formed therefrom.

Desirable commercial requirements for such heat treatable titanium sheet alloy material, for example, are that:

(a) The material in the dead soft, solution treated condition at room temperature should have a maximum ultimate tensile strength of 120,000 p. s. i., a maximum yield strength of 110,000 p. s. i., a minimum elongation of 15%, a maximum bend ductility of 2T, uniform elongation of 10%, and a maximum ratio of 0.9 of yield strength to ultimate strength;

(b) The material should be capable of being aged by heat treatment at a temperature in the neighborhood of 1000° F. and preferably for less than eight hours to develop at room temperature a minimum ultimate tensile strength of 170,000 p. s. i., a minimum yield strength of 155,000 p. s. i., and an elongation of 10%; and

(c) The material at a temperature of 800° F. and after solution treating and aging should have an ultimate tensile strength of 115,000 p. s. i. and a yield strength of 87,000 p. s. i. and must be able to withstand 35,000 p. s. i. at 800° F. for 500 hours and deform no more than 1% under such conditions.

We have discovered that the desired combination of properties may be obtained in sheet alloys of the present invention and that the best combination of most desirable properties may be obtained in a titanium base alloy containing substantially 15% V and 2½% Al. These alloys have excellent forming properties as solution treated in the alpha-beta field or the beta field, and subsequently can be aged to very high strength levels.

The improved titanium-vanadium-aluminum alloys of the present invention have relatively low strength levels and an unusually large spread—up to about 71,000 p. s. i.—between yield strength and ultimate strength as solution treated in the alpha-beta field or the beta field. The ternary titanium base alloy containing 15% V and 2½% Al exhibits the best combination of low strength, a high spread between yield strength and ultimate strength, and high ductility in the solution treated condition. Fur-

2

thermore, the titanium-vanadium-aluminum alloys of the present invention may be subjected to a simple aging treatment to substantially double the ultimate strength and to increase the yield strength by as much as 110,000 p. s. i.

5 Furthermore, we have discovered that the titanium-vanadium-aluminum alloys of the present invention having the indicated properties are further characterized by having excellent uniform elongations as well as high elongation values. Normally titanium alloys do not exhibit 10 uniform elongation, and the provision of a highly ductile titanium alloy having high uniform elongation values is unusual. Uniform elongation is measured in the portion of the gage length of the tensile specimen outside the necked-down area.

For instance, when a sheet tensile specimen is subjected to a tensile test and is pulled, titanium alloys usually neck inward sharply and fail in a short length of the specimen between the gage marks. However, sheet tensile specimens made from the improved alloys of the present invention, when subjected to tensile tests do not necessarily fail between the gage marks but sometimes fail beyond the same. Furthermore, areas within the range of the gauge marks—which were initially marked with ¼" squares—elongated the square markings about 25% in all ½" sections of the specimen.

25 Thus, sheet material formed from the improved titanium alloys of the present invention and having the high uniform elongation values described stretch more or less uniformly over the entire area under stress. Uniform elongation is important in forming operations as it is an indication of how much forming can be done on a part, before "necking down" takes place. The achievement of this characteristic is very important since it provides a kind of ductility permitting the material to be subjected to complicated forming, stamping or deep drawing operations.

30 Accordingly, it is a general object of the present invention to provide a new heat treatable titanium-vanadium-aluminum sheet alloy which may be solution treated to permit forming while highly ductile at low strength levels and thereafter aged to extremely high strength levels.

35 Also, it is an object of the present invention to provide a new titanium-vanadium-aluminum sheet alloy which may be heat treated by heating and quenching to very low strength levels, with reasonably high ductility and excellent formability.

40 It is another object of the present invention to provide a titanium-base vanadium-aluminum sheet alloy which as solution treated in the alpha-beta field or the beta field is highly ductile and at the same time exhibits high uniform elongation values.

45 Another object of the present invention is to provide a titanium-base vanadium-aluminum sheet alloy in which the ultimate strength may be increased as much as twice by a simple aging treatment after forming.

50 Still another object of the present invention is to provide a titanium-base vanadium-aluminum sheet alloy having a desirable combination of low strength, a large spread between yield strength and ultimate strength, and high ductility in the solution treated condition.

55 Finally, it is an object of the present invention to provide a new ternary titanium-vanadium-aluminum sheet alloy and particularly an alloy of titanium and 15% V and 2½ Al.

These and other objects and advantages apparent to those skilled in the art from the following description and claims, may be obtained, the stated results achieved, and the described difficulties overcome by the discoveries, principles, compositions and alloys which comprise the present invention, the nature of which is set forth below—illustrative of the best modes in which applicants have contemplated applying the principles—and which are particularly and distinctly pointed out and set forth in the appended claims forming part hereof.

Certain of the properties of alloys of the present invention are shown in the drawings in which:

Fig. 1 is a graph illustrating the yield strength, ultimate strength and elongation of alloys of the present invention made with 138 BHN sponge titanium base, solution treated in the beta field as well as solution treated in the beta field and then aged;

Fig. 2 is a graph similar to Fig. 1 of alloys made from 106 BHN sponge titanium base;

erties for achieving the objectives and new results of the invention.

The alloys of the present invention after melting and casting may be processed in the usual manner and forged or rolled to form the desired wrought semi-finished or finished product. For instance, ingots of the improved titanium-vanadium-aluminum alloys may be forged or bloomed to slab form, hot rolled to sheet bar, and the sheet bar hot rolled to form finished sheets, say, .030" thick, at about 1400° F.

Since the alloys of the present invention are intended to be subjected to forming operations in the solution treated condition, it is only necessary that the material have some ductility as hot rolled. Typical data and as hot-rolled physical properties (longitudinal) of .030" sheet rolled from alloys containing 15% vanadium and various amounts of aluminum made from sponge having various strength levels are given in Table I below as follows:

TABLE I  
*As hot rolled physical properties (longitudinal)*

| Heat No. | Nominal Composition | Ultimate Tensile Strength, p. s. i. | Yield Strength (0.2% off-set), p. s. i. | Elongation, Percent in 2" | T-Bend (Long.) | Sponge Hardness, BHN | Beta Transus, ° F. |
|----------|---------------------|-------------------------------------|-----------------------------------------|---------------------------|----------------|----------------------|--------------------|
| DM-342   | 15 V                | 149,700                             | 146,600                                 | 1.4                       | 4.1            | 138                  | 1,450              |
| DM-330   | 15 V-2.5 Al         | 118,900                             | 64,200                                  | 9.2                       | 1.5            | 106                  | 1,430              |
| DM-361   | 15 V-2.5 Al         | 123,300                             | 101,500                                 | 5.2                       | 1.7            | 138                  | 1,450              |
| DM-345   | 15 V-4 Al           | 141,500                             | 46,600                                  | 8.6                       | 2.0            | 106                  | 1,480              |
| DM-334   | 15 V-4 Al           | 137,400                             | 80,200                                  | 6.4                       | 2.5            | 138                  | 1,580              |
| DM-346   | 15 V-6 Al           | 145,000                             | 71,400                                  | 8.2                       | 1.9            | 106                  | 1,620              |
| DM-349   | 15 V-6 Al           | 128,100                             | 113,900                                 | 6.2                       | 3.3            | 138                  | 1,620              |

Fig. 3 is a graph similar to Fig. 1 of alloys made from 138 BHN sponge titanium base but solution treated in the alpha-beta field; and

Fig. 4 is a graph similar to Fig. 3 of alloys made from 106 BHN sponge titanium base solution treated in the alpha-beta field.

The alloys of the present invention may be prepared from either commercial titanium or high purity titanium. Where prepared from commercial titanium, a typical analysis of the material in addition to titanium, vanadium and aluminum, is 0.02% C., 0.01% N<sub>2</sub>, 0.10% O<sub>2</sub> and 0.005% H<sub>2</sub>. However, the invention is not restricted to the use of material having the typical interstitial level indicated, as the level may be of the order of 0.06% C., 0.03% N<sub>2</sub>, 0.15% O<sub>2</sub> and 0.019% H<sub>2</sub>. In other words presently available sponge having an average sponge hardness of 120 BHN is suitable and this hardness may fall in the range of 106 BHN to 138 BHN. Thus, in examples given below, titanium sponge having different typical interstitial levels was used such as 106 BHN and 138 BHN sponge.

In practice, the titanium is preferably melted by the electric arc process in a water-cooled copper crucible in a vacuum or an atmosphere such as argon and the alloying elements are added to the melt either as chemically pure components or in the form of a high purity vanadium-aluminum alloy. The latter is preferable because the commercial master vanadium-aluminum alloy available is substantially cheaper in cost than pure vanadium. Also, the master alloy is well adapted without further additions of either vanadium or aluminum to form the preferred 15 V-2.5 Al alloy with titanium.

In general, the alloys of the present invention comprise from 12 to 20 percent vanadium and from 1 to 4 percent aluminum, the balance being all titanium. More particularly, the preferred alloys of the present invention comprise from 14 to 16 percent vanadium and from 2 to 3½ percent aluminum, the balance being all titanium. A 15% V-2½% Al alloy with the balance being all titanium is preferred as it exhibits the best combination of prop-

40 The beta transus temperatures listed in Table I were determined from .080" sheet; and although some discrepancies in these temperatures may be noticed, there is an average 20° F. increase in the transus in going from 106 to 138 BHN sponge, and an increase of about 40° F. for each percent aluminum added.

45 The physical properties of the heats listed in Table I in the solution treated and solution-treated-and-aged conditions are shown graphically in Figs. 1 to 4. Solution treatment temperatures were selected 50° F. above and 75° F. below the beta transus, respectively, for solution treatment in the beta field and solution treatment in the alpha-beta field. After heating, the specimens were water quenched to retain the phase at which solution treatment takes place. All specimens in the aged condition were aged twenty-four hours at 900° F. and then air cooled, which should over-age these alloys.

50 The beta-quenched graphs are indicated at B-1, B-2 and B-3 in Figs. 1 and 2 illustrating, respectively, ultimate tensile strength, yield strength, and elongation values; and corresponding beta-quenched and aged graphs are indicated at B-1A, B-2A and B-3A in Figs. 1 and 2. Similarly, alpha-beta quenched graphs are indicated at AB-1, AB-2 and AB-3 in Figs. 3 and 4, the alpha-beta quenched and aged graphs being indicated at AB-1A, AB-2A and AB-3A in Figs. 3 and 4.

55 In general, referring to Figs. 1, 2, 3 and 4, the higher interstitial level gives higher strength levels after aging. Compare graphs B-1A and B-2A for 138 BHN sponge of Fig. 1 with similar graphs of Fig. 2 of material made from 106 BHN sponge. Solution treated properties show little difference sponge lots.

70 The alloys show low strength levels (see graphs B-1 and B-2 and AB-1 and AB-2 in Figs. 1 to 4) and an unusually large spread between yield strength and ultimate strength as solution treated in either the alpha-beta field or the beta field. Note the distance between graphs B-1 and B-2 in Figs. 1 and 2 and between graphs AB-1 and AB-2 in Figs. 3 and 4 in the range of from 1 to 4 percent aluminum.

The 15 V-2.5 Al-Ti composition exhibits the best combination of low-strength (graphs B-1 and B-2 and AB-1 and AB-2), high yield strength to ultimate strength spread, and high ductility (graphs B-3 and AB-3) in the solution treated condition.

The maximum ultimate tensile strength in each instance is very close to the 120,000 p. s. i. requirement given above, but the maximum yield strength in every instance is far below the 110,000 p. s. i. maximum specified requirement. Similarly the elongation value in each instance is near to the 15% requirement, but the ratio of yield strength to ultimate strength is far below the required 0.9 maximum value.

The high elongation values exhibited by the 15 V-2.5 Al-Ti alloys are also uniform elongations, uniform elonga-

Sheets rolled from the improved alloys may be formed, as by stamping, deep drawing and the like into products or articles of the desired configuration after solution treatment, and such formed parts are subsequently aged to develop the high strength levels therein desired.

The stability of the beta quenched condition at ambient temperatures is shown in the following Table III for aging times of 50 and 100 hours. The results indicate that the yield strength is increased about 20,000 p. s. i. after 50 and 100 hours aging while the ultimate strength and elongation values remain about the same. However, the uniform elongation, particularly after 100 hours, is not as good as in the quenched condition. In use, if this slight age-hardening proves undesirable, the sheet should be solution-treated just before forming.

TABLE III  
Stability tests on the solution treated 15 V-2.5 Al-Ti Alloy

| Aging Time at 150° F., Hrs. | Dir. | UTS, p. s. i. | YS, p. s. i. (0.2% Offset) | Elong., percent in 2" | T-Bend |      | Uniform Elonga-tion, Percent in 1/2" |
|-----------------------------|------|---------------|----------------------------|-----------------------|--------|------|--------------------------------------|
|                             |      |               |                            |                       | L      | T    |                                      |
| 0-----                      | L    | 101,900       | 39,300                     | 15.6                  | 1.8    | 1.8  | 6.3 12.5 18.8                        |
|                             | T    | 100,700       | 43,200                     | 29.7                  | -----  | 21.9 | 28.1 28.1                            |
| 50-----                     | L    | 101,800       | 58,500                     | 14.8                  | 1.1    | 2.6  | 6.3 9.4 12.5                         |
|                             | T    | 97,800        | 62,200                     | 17.2                  | -----  | 20.3 | 23.4 18.8                            |
| 100-----                    | L    | 99,900        | 57,300                     | 14.4                  | 1.3    | 17.2 | 6.3 6.3                              |
|                             | T    | 98,800        | 65,200                     | 25.8                  | -----  | 23.4 | 9.4 9.4                              |

gation being measured in the portion of the gage length of the tensile specimen outside the necked-down area. The 15 V-2.5 Al-Ti alloy has a 29.7% total elongation in 2" while the percent elongation in 1/2" gage sections was 21.9, 28.9 and 28.1. Such uniform elongation values are much greater than the indicated requirement.

The high ductility and large spread between yield and ultimate strength in the solution treated 15 V-2.5 Al-Ti alloy indicates good forming characteristics. The exact explanation of the reasons why these particular properties are developed is not clear, although there is evidence leading to the conclusion that the properties may be attributed to a martensitic reaction occurring during stressing. First, the 15 V-Ti binary has barely enough V to be quenched to retained beta, and the addition of Al apparently makes the alloy a borderline case between a beta-stabilized alloy and a martensitic titanium alloy. Second, the as-beta quenched microstructure is clear beta but develops a martensitic structure after tensile testing.

As indicated in the graphs, aging the solution treated alloys of the present invention results in high strength levels and low elongation. Quenching from the alpha-beta field gives slightly higher aged ductility and somewhat lower strength levels. The lower interstitial level seems to give higher ductility.

Typical annealed properties of the 15 V-2.5 Al-Ti alloy are given in Table II below:

The alloys of the present invention have good solution treated properties even when beta quenched. The 15 V-2.5 Al-Ti alloy exhibits the best combination of properties. It has good solution treated properties even when beta quenched and fair ductility at aged strength levels of 150,000 to 200,000 p. s. i. UTS. The alloy sheet has excellent uniform elongation and a large spread between yield strength and ultimate strength in the solution treated condition. As beta quenched, the 15 V-2.5 Al-Ti sheet is fairly stable up to one hundred hours at 150° although some loss of uniform elongation occurs. To summarize, typical physical properties of .030" sheet made from the 15 V-2.5 Al-Ti alloy, are as follows:

| 45 | Condition                                | UTS, p. s. i. | 0.2% YS, p. s. i. | Percent EL. (2") | T-Bend |   |
|----|------------------------------------------|---------------|-------------------|------------------|--------|---|
|    |                                          |               |                   |                  | I      | T |
| 50 | Solution Treated-----                    | 95,000        | 40,000            | 15-25            | 1-2    |   |
|    | Solution Treated and aged (900° F.)----- | 175,000       | 160,000           | 4                | 5-10   |   |

Such properties provide sheet material having excellent formability in the solution treated condition.

In a series of tests comparing the unusual uniform elongation characteristics of the 15 V-2.5 Al-Ti alloy of the present invention with the uniform elongation values

TABLE II  
Annealed properties of 15 V-2.5 Al-Ti .040" sheet

| Heat Treatment                                      | Dir. | UTS, p. s. i. | YS, p. s. i. (0.2% Offset) | Elong., Percent in 2" | Bend  |       |
|-----------------------------------------------------|------|---------------|----------------------------|-----------------------|-------|-------|
|                                                     |      |               |                            |                       | I     | T     |
| 1,250° F.-1/2 hr.-FC to 900° F.-AC-----             | L    | 124,500       | 106,700                    | 8.2                   | 1.6   | ----- |
| 1,250° F.-1/2 hr.-FC to 900° F.-AC-----             | T    | 130,700       | 114,200                    | 8.2                   | ----- | 2.6   |
| 1,250° F.-1/2 hr.-FC-900° F.-AC, 800°-1 hr.-AC----- | L    | 123,500       | 107,600                    | 7.8                   | 1.3   | ----- |
| 1,250° F.-1/2 hr.-FC-900° F.-AC, 800°-1 hr.-AC----- | T    | 131,200       | 116,400                    | 8.2                   | ----- | 2.6   |

In general, these alloys can be quenched to a clear beta microstructure and aging tends to bring out a fine alpha precipitate. Increasing additions of aluminum to the alloys tends to give a massive alpha precipitate at the prior beta grain boundaries, after aging.

of other titanium alloys which had appeared promising in this respect, the 15 V-2.5 Al-Ti alloy sheet showed very good uniform elongation properties in both the longitudinal and transverse direction in the solution treated condition and showed by far the best uniform elongation

characteristics of all of the alloys checked in the solution treated condition.

The uniform elongation curves for both transverse and longitudinal sheet test specimens of the new 15 V-2.5 Al-Ti alloy show a minimum of 10% uniform elongation with several plateaus showing greater uniform elongation. One of the plateaus for both transverse and longitudinal specimens is above 20% uniform elongation. However, the improved alloy shows poor uniform elongation in the solution treated and aged condition.

These tests were conducted on standard .040" strip tensile specimens with straight reduced sections (i. e., no taper was machined in the gage length). The tensile specimens were marked with a  $\frac{1}{8}$ " square grid over the 2" gage length. The specimens were pulled, using a constant strain rate of .005-in./in./min. to a point past the .2% offset yield point. The percent elongation for each  $\frac{1}{8}$ " was calculated, and a graph using the percent elongation for the ordinate and the length along the 2" gage length as the abscissa was plotted for each specimen.

The shape of the curve formed was the determining factor as to whether the uniform elongation was considered to be good or poor. A curve with plateaus and not jagged peaks was considered to show good uniform elongation.

The strength levels of these .040" sheet tensile specimens tested in the solution treated and in the solution treated and aged conditions were as follows:

| Condition                      | Average UTS, p. s. i. | Average 0.2% YS, p. s. i. | Percent El. (2") |
|--------------------------------|-----------------------|---------------------------|------------------|
| Solution treated.....          | 102,000               | 48,000                    | 16-21.6          |
| Solution treated and aged..... | 188,000               | 172,000                   | 2.7-4.1          |

In making these uniform elongation tests, the solution treatment included heating at 1370° F. for one-half hour and then water-quenching, and the aging involved heating solution-treated material at 900° F. for twenty-four hours and then air cooling.

Although the alloys of the present invention have been described particularly as sheet alloys, the use of the same is not limited to the manufacture of sheet material as the unusual properties can be availed of in other kinds of rolled or forged semi-finished or finished titanium alloy products, herein termed wrought products.

It is to be understood that in the foregoing tables, where intended composition is indicated, there may be some small variation in actual composition determined by chemical analyses. Compositions usually are close to the nominal or intended composition but may vary slightly either way from the intended values, depending upon the ability to control the exact amount of alloying additions made and upon the exact proportions of aluminum and vanadium in the Al-V master alloy which may be used.

The sheet alloys of the present invention accordingly provide a heat treatable material that may be solution treated to low strength levels with reasonably high ductility and a large spread between yield strength and ultimate tensile strength, thereby providing excellent formability. The solution treated or solution treated and formed material may then be aged to high strength levels.

In the foregoing description, certain terms have been used for brevity, clearness and understanding; but no unnecessary limitations are to be implied therefrom beyond the requirements of the prior art, because such terms are utilized for descriptive purposes herein and not for the purpose of limitation and are intended to be broadly construed.

Having now described the invention, the features, discoveries and principles thereof, the characteristics of the new alloys, and the new and useful results obtained, the new and useful compositions, combinations, products, discoveries, and principles, and reasonable mechanical

equivalents thereof obvious to those skilled in the art are set forth in the appended claims.

We claim:

- 5 1. A rolled heat treated titanium base alloy sheet product formed of a titanium base alloy consisting of 14% to 16% vanadium, 2% to 3½% aluminum, and the balance titanium with incidental impurities; said product being characterized by having in the solution-treated condition a ratio of yield strength to ultimate tensile strength from about 0.9 to as low as 0.5, an ultimate tensile strength less than 120,000 p. s. i., elongation in excess of 15%, and uniform elongation in excess of 10%.
- 10 2. A rolled heat treated titanium base alloy sheet product formed of a titanium base alloy consisting of 14% to 16% vanadium, 2% to 3½% aluminum, and the balance titanium with incidental impurities; said product being characterized by having in the solution-treated condition a ratio of yield strength to ultimate tensile strength from about 0.9 to as low as 0.5, an ultimate tensile strength less than 120,000 p. s. i., elongation in excess of 15%, and uniform elongation in excess of 10% permitting forming of the sheet product at such low strength levels; and said sheet product having an ultimate tensile strength of from 150,000 to 200,000 p. s. i. when aged at 900° F. after solution treatment.
- 15 3. A wrought heat treated titanium base alloy product formed of a titanium base alloy consisting of 14% to 16% vanadium, 2% to 3½% aluminum, and the balance titanium with incidental impurities incident to the use of commercial titanium sponge having a hardness in the range of 106 to 138 BHN; said product being characterized by having in the solution-treated condition a ratio of yield strength to ultimate tensile strength from about 0.9 to as low as 0.5, an ultimate tensile strength less than 120,000 p. s. i., elongation in excess of 15%, and uniform elongation in excess of 10% permitting forming of the product at such low strength levels; and said product having an ultimate tensile strength of from 150,000 to 200,000 p. s. i. when aged at 900° F. after solution treatment.
- 20 4. A rolled heat treated titanium base alloy sheet product formed of a titanium base alloy consisting of 15% vanadium, 2½% aluminum, and the balance titanium with incidental impurities; said product being characterized by having in the solution-treated condition a yield strength as low as 40,000 p. s. i., an ultimate tensile strength less than 120,000 p. s. i. to as low as 95,000 p. s. i., a ratio of yield strength to ultimate tensile strength from about 0.9 to as low as 0.5, elongation of from 15% to 25%, and uniform elongation in excess of 10% permitting forming of the sheet product at such low strength levels; and said sheet product having a yield strength in excess of 160,000 p. s. i. and an ultimate tensile strength in excess of 175,000 p. s. i. when aged at 900° F. after solution treatment.
- 25 5. A rolled heat treated titanium base alloy sheet product formed of a titanium base alloy consisting of 14% to 16% vanadium, 2% to 3½% aluminum, and the balance titanium with incidental impurities; said product being characterized by having in the solution-treated condition a ratio of yield strength to ultimate tensile strength from about 0.9 to as low as 0.5 with a spread of up to 71,000 p. s. i. between yield strength and ultimate tensile strength, elongation in excess of 15%, and uniform elongation in excess of 10%; and said sheet product having an ultimate tensile strength of from 150,000 to 200,000 p. s. i. when aged.
- 30 6. A rolled heat treated titanium base alloy sheet product formed of a titanium base alloy consisting of 14% to 16% vanadium, 2% to 3½% aluminum, and the balance titanium with incidental impurities; said product being characterized by having in the solution-treated condition a ratio of yield strength to ultimate tensile strength from about 0.9 to as low as 0.5 with a spread of up to 71,000 p. s. i. between yield strength and ultimate tensile strength,
- 35
- 40
- 45
- 50
- 55
- 60
- 65
- 70
- 75

elongation in excess of 15%, and uniform elongation in excess of 10%; and said sheet product when aged having an ultimate tensile strength substantially twice that of its ultimate tensile strength in the solution-treated condition and a yield strength increased as much as 110,000 p. s. i. from the yield strength of the product in solution-treated condition.

5

## References Cited in the file of this patent

## UNITED STATES PATENTS

2,754,204 Jaffee et al. ----- July 10, 1956

## FOREIGN PATENTS

1,094,616 France ----- Dec. 8, 1954

**Disclaimer**

2,864,697.—*Lee S. Busch, George W. Bauer and Paul E. Moorhead*, Warren, Ohio. TITANIUM-VANADIUM-ALUMINUM ALLOYS. Patent dated Dec. 16, 1958. Disclaimer filed July 13, 1966, by the assignee, *National Distillers & Chemical Corporation*.

Hereby enters this disclaimer to claims 1 through 6 inclusive of said patent.

[*Official Gazette August 23, 1966.*]